# EUROPEAN PATENT SPECIFICATION

(11) **EP 0 292 780 B1**
(45) Date of publication and mention of the grant of the patent: **14.11.1990**
(21) Application number: 88107511.3
(22) Date of filing: 10.05.1988
(51) Int. Cl.: H01B 7/34, H01B 7/28, H01B 3/10, H01B 13/06

(54) **Electric wire**
Elektrischer Draht
Fil électrique

(30) Priority: 12.05.1987 JP 115576/87
(43) Date of publication of application: 30.11.1988
(73) Proprietor: SUMITOMO ELECTRIC INDUSTRIES, LTD., Osaka-shi, Osaka 541 (JP)
(72) Inventor: Inazawa, Sinji Osaka Works, Konohana-ku Osaka (JP); Sawada, Kazuo Osaka Works, Konohana-ku Osaka (JP)
(74) Representative: Patentanwälte Kirschner & Grosse

(56) References cited:
- EP-A- 0 170 441
- EP-A- 0 188 369
- EP-A- 0 188 370

## Description

### BACKGROUND OF THE INVENTION

### Field of the Invention

The present invention relates to an electric wire, and more particularly, it relates to an electric wire which is applied to an electric wire requiring fire resistance and heat resistance such as a magnet wire or a wire employed in the vicinity of a nuclear reactor, or a special wire or cable requiring corrosion resistance.

### Description of the Prior Art

The aforementioned electric wire requiring heat resistance or corrosion resistance is generally prepared by a covered conductor, which is coated with organic material. However, an organic coating film is insufficient in long-term stability, heat resistance, chemical durability and the like.

Thus, there has been provided a conductor coated with a compound of metal or metalloid, which is different from the material for the conductor, in order to attain heat resistance and corrosion resistance. For example, National Patent Publication Gazette No. 501783/1985 in the name of Raychem Inc., published in Japan on October 17, 1985, discloses a conductor which is coated with an oxide or a nitride by vacuum deposition, in order to provide heat resistance to an electric wire to be utilized under a high temperature. A compound for forming such coating is prepared by an oxide or a nitride of aluminum, silicon etc. Since such oxide is excellent in heat resistance and corrosion resistance, an electric wire coated with the oxide can be provided with high heat resistance and corrosion resistance.

The aforementioned electric wire which is covered with a ceramic film has been studied for improving these characteristics. Such a ceramic film is formed by:
(a) a method of forming a film from a vapor phase (vapor phase thin film growth method), such as CVD (chemical vapor deposition), PVD (physical vapor deposition) or flame coating;
(b) an electrochemical method of forming a film in a solution, such as plating;
(c) a sol-gel method of forming a film from a liquid phase by chemical reaction of reacting alkoxide; or
(d) a method of forming a film by dipping in a melt.

As hereinabove described, it is well known that an oxide of ceramics such as A1₂0₃ or Si0₂ is excellent in heat resistance and corrosion resistance. However, such an oxide formed by vacuum deposition is rather insufficient in adhesion to the material, such as copper, for a conductor. Therefore, when an electric wire coated with an oxide is used under corrosive environment over a long period of time, for example, the oxide film may partially peel off from the copper surface, to result in corrosion from the exposed portion.

The vapor phase thin film growth method such as vacuum deposition is employed as a method of forming an oxide film on the surface of a conductor. However, a film obtained by vacuum deposition or the likeway be inferior in flexibility. Therefore, when a wire coated with an oxide by vacuum deposition is used in a bended state, for example, the oxide film may be broken by stress applied to the surface of the conductor, to result in corrosion from the broken portion.

EP-A 188 370 describes an electrical wire comprising a copper conductor and an electrical insulating refractory coating. At least part of the coating and preferably alll the coating has been formed by a sol-gel method. In addition, the conductor includes a keying layer formed from a metal other than copper in order to icnrease the adhesion of the refractory coating to the conductor.

### SUMMARY OF THE INVENTION -

Accordingly, an object of the present invention is to provide an electric wire which effectuates excellent heat resistance and corrosion resistance over a long period of time, by forming a film having excellent adhesion and flexibility. Another object of the present invention is to provide an electric wire which can be industrially obtained by simple means in a step of coating an elongated wire conductor.

An electric wire in accordance with the present invention comprises a conductor and at least one coating of a film obtainable by applying a gel obtained by hydrolyzing and condensing an alkoxide on an outer part of said conductor, characterized by leaving said gel film after it has been applied to the conductor in a state in which it is not completely changed into condensed oxide.

The gel film contributing to heat resistance, which is formed by a sol-gel method in the present invention, is excellent in flexibility and adhesion since the same is left not to be completely changed into a ceramic state but to remain in a gel state. This gel film is changed into a ceramic state by heating, to be improved in heat resistance. However, it has been recognized that its flexibility is reduced as much as it is changed into a ceramic state. On the basis of such a viewpoint of the inventors, the gel film is formed as a main heat resisting layer in the present invention. The conductor is preferably left in an atmosphere being at a temperature not less than 25_{°}C, not more than 400_{°}C, in order to form the gel film as a main heat resisting layer.

When the outer surface of a conductor coated with the solution obtained by hydrolyzing and dehydrating/condensing alkoxide and left is oxidized by heat, an oxide thus produced is so fragile that adhesion between the gel film and the conductor surface is lost to cause peeling of the film. In order to prevent this, the conductor surface is preferably plated with Ni or Cr for attaining oxidation resistance, before the same is coated with the solution and left in the aforementioned manner.

Upon heating, the gel film is considerably shrunk to be reduced in thickness. Such shrinkage of the film may result in inferior durability of insulation. While a conductor subjected to low voltage may be simply coated with a gel film alone, a problem is caused in durability of insulation when such a simple coated wire is applied to a power cable. Therefore, particulates of a metal oxide, a metal nitride or a metal boride are preferably dispersed/mixed in the gel film as ceramic filler for suppressing shrinkage of the gel film. Although the gel film is considerably flexible in a natural state, such flexibility may be lost when the gel film is heated to be changed into a ceramic state. Even if the electric wire is utilized in a portion exposed to strong vibration, the film changed into a ceramic state must not peel off from the conductor by cracking caused by the strong vibration. Thus, particularly strong adhesion may be required between the gel film and the conductor. In this case, an adhesion layer may be provided between the gel film and the conductor, or between the gel film and a plating layer formed on the surface of the conductor. The adhesion layer may be prepared by a film completely changed into a ceramic state by applying a solution obtained by hydrolyzing and dehydrating/condensing alkoxide and thereafter heating the same. Alternatively, the adhesion layer may be prepared by a ceramic layer formed by CVD, on the basis of such a viewpoint of the inventors that a layer formed by CVD is larger in adhesion to a substrate than a gel film.

The inventive wire may be provided with an outermost layer of organic material, in order to improve slipperiness in winding and durability of insulation under the room temperature. In this case, the particulates of a metal oxide etc. may be dispersed/mixed in the organic material layer to improve durability of insulation.

Further, the organic material layer may be formed from a solution of organic material, added to which is a solution obtained by hydrolyzing and dehydrating/condensing alkoxide with addition of tetraalkylammonium halide to be mixable into the solution of organic material, in order to improve heat resistance.

A gel film in accordance with the present invention may be formed as a multilayer film having two or more layers, in order to improve heat resistance, corrosion resistance and durability of insulation. In the process of forming the gel film in accordance with the present invention, alkoxide may be hydrolyzed by moisture contained in the atmospheric air, without directly adding water to an alkoxide solution.

These and other objects, features, aspects and advantages of the present invention will become more apparent from the following detailed description of the present invention when taken in conjunction with the accompanying drawings.

### BRIEF DESCRIPTION OF THE DRAWINGS

Figs. 1 A, 1 B, 1 C and 1D are sectional views showing electric wires in accordance with the present invention; and
Fig. 2 illustrates an apparatus for performing a heat resistance test on samples of the electric wires in accordance with the present invention.

### DESCRIPTION OF THE PREFERRED EMBODIMENTS

Figs. 1 A to 1 D are sectional views showing electric wires in accordance with the present invention.

Fig. 1A shows an electric wire, which comprises a conductor 1 of copper etc. coated with a gel film 2 of one or more layers. Fig. 1B shows an electric wire which comprises a conductor 1, a-plating layer 3 of Ni or Cr formed on the surface thereof, a gel film 2 covering the plating layer 3 and a covering layer 6 of organic material. Fig. 1 C shows an electric wire which has a gel film 2 and a ceramic film 4 formed under the gel film 2 by CVD to serve as an adhesion layer. Fig. 1D shows an electric wire which has a ceramic film 5 formed by a starting raw material of alkoxide, to serve as an adhesion layer. This ceramic film 5 is formed by applying a solution obtained by hydrolyzing and dehydrating/condensing metal alkoxide and thereafter heating the same.

Samples for a heat resistance test of the aforementioned electric wires embodying the present invention were prepared as follows: Each of coating solutions 1 to 6, being prepared by the following methods, was applied onto a copper wire of 2.0 mm in diameter by a dipping method at a lift-up speed of 1.0 m/min., to form a multilayer film on the copper wire.

### Coating Solution 1

Tetrabutylorthosilicate [Si(OC₄H₉)_{4]}, isopropyl alcohol [C₃H₇OH] and water [H₂0] were mixed in the mole ratio 10:50:40 to obtain a solution, to which nitric acid was added by 1/100 mol of tetrabutylorthosilicate. Then the solution was stirred at a temperature of 80_{°}C for 100 minutes, and thereafter returned to the room temperature.

### Coating Solution 2

Tetraethylorthosilicate [Si(OC₂Hs)4], ethyl alcohol [C₂HₛOH] and water [H₂O] were mixed in the mole ratio 3:60:37 to obtain a solution, to which nitric acid was added by 1/100 mol of tetraethylorthosilicate. Then the solution was stirred at a temperature of 70_{°}C for 100 minutes, and thereafter returned to the room temperature.

### Coating Solution 3

Tetrabutylorthosilicate [Si(OC₄H₉)₄], isopropyl alcohol [C₃H₇0H] and water [H₂0] were mixed in the mole ratio 20:60:20 to obtain a solution, to which nitric acid was added by 1/100 mol of tetrabutylorthosilicate. Then the solution was stirred at a temperature of 80_{°}C for 200 minutes, and thereafter returned to the room temperature.

### Coating Solution 4

Tetrabutylorthosilicate [Si(OC₄H₉)₄], isopropyl alcohol [C₃H₇0H] and water [H₂0] were mixed in the mole ratio 10:50:40 to obtain a solution of 100 g, to which silicagel by Wako Junyaku (WAKOGEL, C-100) of 30 g was previously added. Then nitric acid was added by 1/100 mol of tetrabutylorthosilicate, and the solution was stirred at a temperature of 80°C for 100 minutes, and thereafter returned to the room temperature.

### Coating Solution 5

### p-xylene 30% solution of polyimide

### Coating Solution 6

Tetrabutylorthosilicate [Si(OC₄H₉)₄], isopropyl alcohol [C₃H₇0H] and water [H₂0] were mixed in the mole ratio 10:50:40 to obtain a solution, to which nitric acid was added by 1/100 mol of tetrabutylorthosilicate. Then the solution was stirred at a temperature of 80°C for 100 minutes and thereafter returned to the room temperature. Tetrabutylammonium bromide [(C₄H₉)₄N⁺Br] of 20 g was added to the solution of 100 g and stirred with addition of chloroform [CHCl₃], to perform extraction.

This extract was decompressed/dried by an evaporator to remove the solvent, thereby to obtain a pale yellow consistent liquid [SiO₂ polymer]. This SiO₂ polymer was mixed into 10 ml of a p-xylene 30% solution of polyimide, which was then stirred under the room temperature.

Each of the coating solutions 1 to 6 was employed for coating, to form a film by the following treatment. Thus, samples A, B, C, D, E and F were obtained by copper wires having multilayer coating films at least including gel films, as shown in Tables 1 to 6.

Heat Resistance Test

Insulation Test: As shown in Fig. 2, two samples 7a and 7b were brought into contact with each other to be heated by a heater 12 at a prescribed temperature for 30 minutes with application of voltage of 50 V, thereby to confirm insulating performance.

Vibration Test: In the insulation test, a motor 15 as shown in Fig. 2 was rotated with a dead weight 16 of 5 g, to apply vibration.

Referring to Fig. 2, numerals 7a and 7b indicate the samples, numeral 8 indicates a quartz plate on which the samples 7a and 7b are placed to be in contact with each other, and numeral 9 indicates a quartz pipe for storing the samples 7a and 7b placed on the quartz plate 8, having an end sealed by a closure 10 of silicon rubber and another end blocked by a glass wool member 11. A heater 12 prepared by a tube furnace is provided around the quartz pipe 9, in order to heat the samples 7a and 7b. A thermocouple 13 is inserted into the quartz pipe 9 through the closure 10, in order to measure the temperatures of the samples 7a and 7b. Numerals 14a and 14b indicate lead wires, which are connected to the samples 7a and 7b respectively, to be linked to electrodes for the insulation test. The motor 15 is provided on an end of the quartz plate 8 outwardly extending from the quartz pipe 9 through the glass 9 wool member 11, in order to apply vibration to the samples 7a and 7b. The dead weight 16 of 5 g is mounted on the shaft of the motor 15, which is rotated to vibrate the quartz plate 8, thereby to transfer the vibration to the samples 7a and 7b. A support 17 is provided in order to support the quartz plate 8.

Table 7 shows the results of such a heat resistance test with characteristics of the respective samples under the room temperature. Referring to Table 7, "x mmd" shows the value of a diameter which caused no abnormality in the coated layer when the copper wire of each sample was wound on a rod of x mm in diameter in a bending test. Table 7 also shows voltage resistance (V). Table 7 further shows results of insulation-sustainable temperature (_{°}C) and vibration-proof temperature (_{°}C). The "insulation-sustainable temperature" indicates the maximum temperature capable of sustaining insulating performance and the "vibration-proof temperature" indicates the maximum temperature capable of sustaining insulating performance against the vibration applied in the aforementioned manner.

It is understood from the result of the insulation test that the electric wire in accordance with the present invention is excellent in flexibility and its insulating performance can be maintained under a high temperature.

## Claims

1. An electric wire comprising a conductor and at least one coating of a film obtainable by applying a gel obtained by hydrolyzation and condensation of an alkoxide directly or indirectly on an outer part of said conductor, characterized by leaving said gel film after it has been applied to the conductor in a state in which it is not completely changed into condensed oxide.

2. An electric wire in accordance with claim 1, wherein said leaving is performed in an atmosphere being at a temperature not less than 25°C, not more than 400_{°}C.

3. An electric wire in accordance with claim 1, wherein said conductor is provided on its surface with a plating layer of either Ni or Cr, said coating of said gel film being provided on its outer part.

4. An electric wire in accordance with claim 1, wherein said gel film is formed as a multilayer film having two or more layers.

5. An electric wire in accordance with claim 1, wherein particulates of at least a metal oxide, a metal nitride or a metal boride are dispersed in said gel film.

6. An electric wire in accordance with claim 1, wherein an underlayer of said gel film is an adhesion layer of a ceramic film formed by applying a solution obtained by hydrolyzing and condensing metal alkoxide and thereafter heating the same.

7. An electric wire in accordance with claim 1, wherein an underlayer of said gel film is an adhesion layer of a ceramic film formed by CVD.

8. An electric wire in accordance with claim 1, further including a covering layer of organic material formed on an outer part of said gel film.

9. An electric wire in accordance with claim 8, wherein particulates of at least a metal oxide, a metal nitride or a metal boride are dispersed in said covering layer.

10. An electric wire in accordance with claim 8, wherein said covering layer is formed from a solution of organic material, added to which is a solution obtained by hydrolyzing and condensing alkoxide with addition of tetraalkylammonium halide to be mixable to said solution of organic material.

## Patentansprüche

1. Elektrischer Draht mit einem Leiter und wenigstens einem Überzug aus einem Film, der durch das mittelbare oder unmittelbare Aufbringen eines durch Hydrolyse oder Kondensierung eines Alkoxids gewonnenen Gels auf einem äußeren Teil des Leiters erhalten werden kann, gekennzeichnet dadurch, daß der Gelfilm nach dem Aufbringen auf den Leiter in einem Zustand belassen wird, in dem er nicht völlig in kondensiertes Oxid umgewandelt ist.

2. Elektrischer Draht nach Anspruch 1, wobei das Belassen in einer Atmosphäre bei einer Temperatur von nicht weniger als 25°C und nicht mehr als 400_{°}C durchgeführt wird.

3. Elektrischer Draht nach Anspruch 1, wobei der Leiter auf seiner Oberfläche mit einer Plattierungsschicht entweder aus Ni oder Cr versehen ist, wobei der Überzug aus dem Gelfilm au seinem äußeren Teil vorgesehen ist.

4. Elektrischer Draht nach Anspruch 1, wobei der Gelfilm als mehrschichtiger Film mit zwei oder mehr Schichten gebildet ist.

5. Elektrischer Draht nach Anspruch 1, wobei Teilchen von wenigstens einem Metalloxid, einem Metallnitrid oder einem Metallborid in dem Gelfilm dispergiert sind.

6. Elektrischer Draht nach Anspruch 1, wobei eine Unterschicht des Gelfilms eine Haftschicht aus einem Keramikfilm ist, der dadurch gebildet wird, daß eine durch Hydrolyse und Kondensierung von Metallalkoxid erhaltene Lösung aufgebracht und diese anschließend erhitzt wird.

7. Elektrischer Draht nach Anspruch 1, wobei eine Unterschicht des Gelfilms eine Haftschicht aus einem durch chemische Abscheidung gewonnenen Keramikfilm ist.

8. Elektrischer Draht nach Anspruch 1, der ferner eine auf einem äußeren Teil des Gelfilms gebildete Deckschicht aus organischer Substanz aufweist.

9. Elektrischer Draht nach Anspruch 8, wobei Teilchen von wenigstens einem Metalloxid, einem Metallnitrid oder einem Metallborid in der Deckschicht dispergiert sind.

10. Elektrischer Draht nach Anspruch 8, wobei die Deckschicht aus einer Lösung einer organischen Substanz ausgebildet ist, zu der eine durch Hydrolyse oder Kondensierung von Alkoxid unter Beifügung von Tetraalkylammoniumhalid gewonnene Lösung zugegeben ist, die mit der Lösung der organischen Substanz mischbar ist.

## Revendications

1. Un fil électrique comprenant un conducteur et au moins un enrobage consistant en un film pouvant être obtenu par application d'un gel obtenu par hydrolyse et condensation d'un alkoxyde, directement ou indirectement sur une partie extérieure dudit conducteur, caractérisé par le fait de laisser en place ledit film de gel après l'avoir appliqué sur le conducteur, dans un état dans lequel il n'est par complètement transformé en oxyde condensé.

2. Un fil électrique selon la revendication 1, dans lequel ladite exposition est effectuée dans une atmosphère dont la température n'est pas inférieure à 25_{°}C ni supérieure à 400_{°}C.

3. Un fil électrique selon la revendication 1, dans lequel ledit conducteur est pourvu, à sa surface, d'un revêtement de plaquage soit en Ni soit en Cr; ledit enrobage avec ledit film en gel étant effectué sur sa partie extérieure.

4. Un fil électrique selon la revendication 1, dans lequel ledit film en gel est en forme de film multicou- ches présentant deux couches ou plus.

5. Un fil électrique selon la revendication 1, dans lequel des particules d'au moins un oxyde métallique, un nitrure métallique ou un borure métallique sont dispersées dans ledit film en gel.

6. Un fil électrique selon la revendication 1, dans lequel une sous-couche dudit film en gel est une couche d'adhésion d'un film céramique formé par application d'une solution obtenue par hydrolyse et condensation d'un alkoxyde métallique, suivi d'un chauffage de ce dernier.

7. Un fil électrique selon la revendication 1, dans lequel une sous-couche dudit film en gel est une couche d'adhésion d'un film céramique formé par procédé DPV (dépôt en phase vapeur).

8. Un fil électrique selon la revendication 1, comprenantJen outre-une couche de revêtement en matériau organique formée sur une partie extérieure dudit film en gel.

9. Un fil électrique selon la revendication 8, dans lequel des particules d'au moins un oxyde métallique, un nitrure métallique ou un borure métallique sont dispersées dans ladite couche de revêtement.

10. Un fil électrique selon la revendication 8, dans lequel ladite couche de revêtement est formée à partir d'une solution d'un matériau organique, additionnée d'une solution obtenue par hydrolyse et condensation d'un alkoxyde avec addition d'un halogénure de tétraalkylammonium par mélange à ladite solution de matériau organique.
